

June 6, 1944.

C. H. SCHUH

2,350,422

CORK PRODUCTS AND PROCESS OF MAKING THE SAME

Filed Aug. 7, 1941



BY

INVENTOR.  
*Charles H. Schuh*  
*Sidney A. Ochs*  
ATTORNEY

## UNITED STATES PATENT OFFICE

2,350,422

COKE PRODUCT AND PROCESS OF MAKING  
THE SAMECharles H. Schuh, Ridgewood, N. Y., assignor to  
Carbide and Carbon Chemicals Corporation, a  
corporation of New York

Application August 7, 1941, Serial No. 405,824

14 Claims. (Cl. 202—18)

This invention relates to the treatment of cork materials to obtain low density cork pieces useful, for instance, in insulation and acoustical compositions and products, to the treated cork per se and to by-products of said treatment.

The invention particularly relates to cork granules having a pliable springy character and extremely low density and to a process of producing said cork granules utilizing as a medium of expansion and treatment a liquid bath, for instance of a molten metallic substance preferably comprising lead and which liquid medium is substantially non-absorbent and substantially non-adherent to cork and preferably substantially inert to cork and its decomposition products.

Molten metallic and other liquid baths have heretofore been employed for the destructive distillation of organic materials. For instance, it has been proposed to subject coal, wood, sawdust and shale to destructive distillation in metallic baths, lead containing baths being amongst those employed. The object of the treatment has been to obtain maximum distillation products and the solid residue substances have been by-products or waste products. Examination of such solid residues shows that the substances treated shrink in processing and become brittle, regardless of time and temperature of treatment. It has also been proposed to treat a mineral matter, for instance mica, in such alternative molten mediums as metal or glass to effect an exfoliation of the mica material. Here again control of temperature and time of treatment, insofar as the solid residue is concerned, has not been a consideration, since mica is a mineral that can be subjected to heat for extended periods and to intense temperatures without adverse effects, and in treating this substance once a temperature high enough for exfoliation has been reached the application of higher temperatures or long periods of treatment has no further effect upon the material.

With respect to cork it has heretofore been proposed to expand pieces of natural cork by heating in a gaseous medium, for instance super-heated steam, and to compress the expanded pieces in a mold into a unitary slab, the natural resins of the cork binding the pieces together in the process. According to this procedure, the cork cells are expanded and the cork itself undergoes a loss in density due to the removal of moisture and some decomposition volatile matter. In making molded cork slabs it has been further suggested that the pieces of natural cork be pre-

heated in a receptacle to a temperature between 400° F. to 550° F. or to bring the cork pieces to such temperatures in a lead metallic bath to obtain an increase of volume between 35 to 100 per cent. In this condition the cork pieces retain the relatively hard characteristics of natural cork theretofore used. Subsequently the expanded pieces are compressed in a mold and baked at the conventional baking temperatures at or above 600° F. while retaining the pieces under pressure to consolidate the pieces into unitary bonded slabs.

Insofar as expanding cork pieces in a liquid medium to obtain a large degree of expansion and very low densities without destruction of the cork is concerned, it is believed that these and other prior teachings have suggested this to be impossible. For instance, in United States Letters Patent 997,056 it is taught that the cork pieces should be treated at temperatures below 200° C. (392° F.) when subjected to a liquid bath, as the cork cells are flabby at a high temperature and cannot withstand the pressure of the column of liquid above such temperature. Moreover, Patent 997,056 indicates that when cork is boiled in water or linseed oil and resin that only small expansions are possible and that for any appreciable expansion a gaseous medium should be employed.

In contrast to the prior teachings, I have discovered that with proper precautions and within the critical limitations hereinafter set forth cork pieces may be expanded in a non-absorbent liquid medium, for instance in a molten metallic bath preferably comprising lead, to an extent even considerably beyond that possible in a gaseous medium and with the obtaining of excellent residual properties. I have found that a regranulated cork of even more advantageous properties than that disclosed in my co-pending application Serial No. 271,202 may be made in this manner. The new process differs completely from the process of treating natural cork waste as carried out in a retort or rapid heating of such material with an inert gas in a rotary kiln as described in said prior application, and is simple, quick, more efficient and more economical. Regranulated cork obtained according to the present invention, moreover, permits new features of lower density and greater resiliency to be given to the light weight compositions of such material described in said co-pending application.

Thus, it is amongst the objects of my invention to produce expanded cork pieces by a treatment

in a bath, substantially non-absorbent and non-adherent relative to cork, and to produce expansions of such material even as high as 200 to 375 per cent by volume where the raw material is natural cork. A further object is to produce expanded cork pieces having a density of less than  $2\frac{1}{2}$  pounds and even as low as  $1\frac{1}{2}$  pounds per cubic foot and which expanded cork pieces will have a substantial springy character, be soft and rubbery as distinguished from natural cork and will not possess such an amount of surface carbonization as will produce a brittle surface. Another object is to produce an expanded cork material having a density between about 2 and  $2\frac{1}{2}$  pounds per cubic foot and which cork will retain substantially 80% or more of the original volatile matter in the cork in natural air dried state. A further object is to produce cork granules having a density between  $1\frac{1}{2}$  and 2 pounds per cubic foot and which cork pieces will retain between about 60 to about 80 per cent by weight of the volatiles contained in the cork in natural air dried form, and will have the property of inhibiting fungus growth when combined in sufficient amount with organic substances, for instance cellulose. A further object is to submerge natural or other cork pieces in a molten metallic bath, preferably consisting of lead, for a total period between about 40 seconds to about 4 minutes, the temperature of the bath being maintained between 580° F. to 720° F. but preferably between 620° F. and 680° F. A further object is to pretreat the natural cork or other cork pieces, before treating in a liquid bath as aforesaid, by boiling in water preferably for a period of about 10 minutes to about 30 minutes to cause said cork material to absorb moisture, to thereby obtain maximum expansion of the cork pieces when treated in the liquid bath.

These and further objects of the invention will, in part, be inferred and, in part, appear from the following description and claims and from the drawing illustrating schematically a continuous process for obtaining the products of the invention.

In accordance with the present invention, I have discovered that natural cork pieces (which usually have a density between 6 to 8 pounds per cubic foot when of a size passing a 12 mesh screen and about 55% of the weight of which constitutes volatile and decomposition matter, removable at a temperature between about 620° F. to 680° F.) may be expanded as much as 200 to 375 per cent by volume and be reduced to densities even as low as 1.5 pounds per cubic foot, when submerged in a hot liquid bath substantially non-absorbent and non-adherent to cork, the period of treatment and the temperature range of the bath being within those limits hereinafter given within which the new results may be obtained without destruction of the cork or overburning thereof. At the proposed temperatures of the bath I have found that rapid and optimum expansion of the cork is possible so that an expanded product of lowest density may be obtained in which the cells remain pliable and expanded and are, in fact, more springy than in the original natural cork. Moreover, the temperature permits this expansion to occur without subjecting the cork material to excessive surface carbonization.

I have found that the temperature of the bath for best results should not be much higher than 620° F., preferably within 20° to 35° F. above this temperature, as above about 655° F. cork pieces have a tendency to burn when removed from the

bath and this tendency increases with higher temperatures; also above 655° F. surface carbonization of the cork pieces begins to become substantial. However, good results have also been obtained with temperatures of the bath from above 655° F. to about 680° F. (360° C.) without excessive burning tendency or over carbonization. It has further been found that natural cork granules or pieces of a size not exceeding  $\frac{1}{2}$ " in thickness or passing a  $\frac{1}{4}$  inch to  $\frac{1}{2}$  inch mesh screen will process and obtain maximum expansion in the temperature range 620-655° F. in about 40 seconds. In this exceedingly short period of treatment about 15% to 20% by weight of the cork of volatile and decomposition matter is given off which may be and is preferably condensed and recovered to obtain by-products. The expanded cork material when ground will be found to provide a regranulated cork of about 2 to  $2\frac{1}{2}$  pounds per cubic foot density and between about 40% to 48% of its weight will constitute volatile and decomposition matter that is still removable. The product will be very springy, much more than natural cork; will be soft and rubbery a combination of properties not characteristic of natural cork or of any expanded cork of which I am aware, and will function satisfactorily as a regranulated cork in compositions such as described in my co-pending application aforesaid with improved results. The resultant cork, however, will not have the fungus growth inhibiting properties described in my co-pending application aforesaid as an insufficient amount of decomposition matter is formed in this treatment. However, if treatment of the cork material in the bath be extended past 40 seconds to a period up to about 3 to 4 minutes, depending upon the size of pieces being treated, further distillation of volatile decomposed matter will continue up to about 40% by weight of the original pieces. In this range of treatment between about 25% and 40% by weight of the cork will constitute volatile and decomposition matter still removable and the cork pieces will be found, upon division, to have a density between about  $1\frac{1}{2}$  and about 2 pounds per cubic foot. This cork will also possess soft and rubbery properties and will, further, exhibit fungus growth inhibiting properties. However, it is found that the physical characteristics of the treated cork material begins to undergo some loss in its springy character as the upper time limit of treatment is approached and that if the treatment is continued beyond about 4 minutes there results a brittle surfaced product easily crushed to a powder, and that lacks the desirable properties of the regranulated cork described above which may be put to useful application, for instance in preparing compositions of the character described in my prior application aforesaid. As the ingredient for the bath it is preferred to use a molten metal, for instance lead, tin, bismuth or alloys of, for instance, two or more of lead, zinc, tin, bismuth, antimony, inasmuch as these are non-absorbent in their effect upon cork, may be readily handled and are substantially inert insofar as chemically reacting with the cork or volatiles extracted therefrom during treatment is concerned. I have found molten lead alone to be particularly satisfactory and preferable for use in this invention, inasmuch as it is low in cost, is readily cleansed of impurities and has a melting point within the critical range for best results set forth for this invention, thus making possible a visual control as to the low limit not obtain-

able where an alloy or metal having a melting point outside of the temperature range is utilized. It is to be observed that the use of a lead bath is remarkable when considering the high pressure of this molten material against the expanding cells of the cork and the rapid removal of moisture and decomposition products made possible by such material, and in particular in view of the prior concepts held regarding the use of liquid baths generally in the treatment of cork material.

When the temperature of the bath falls below the melting point of lead (621° F.) such as becomes possible when a lead alloy, for example, is employed and the temperature is not brought up to the desired range, it becomes necessary to extend the period of treatment of the cork pieces to obtain the expanded material. It appears that the heat penetration substantially below such temperature is neither as rapid as that in the preferred range nor does the heat extend completely into the cork of the treated pieces unless the time interval of treatment be considerably extended with a resultant increase in carbonization at the surface and a product having less resiliency. In spite of this condition I have found that cork material of useful character but not as desirable as that obtained in the preferred temperature ranges of treatment is possible with baths having a temperature as low as 580° F. A useful product is also obtained in the temperature range above 680° F. to 720° F. (360° C.), but it has been found that above 680° F. excessive burning of the cork begins to take place. Accordingly, temperatures above 720° F. and below 580° F. should, therefore, be avoided. Also treatment should not exceed about 4 minutes.

The length of time within the prescribed limits to which the cork material is subject to the treatment will be somewhat dependent upon the grade of natural cork employed and the extent of moisture therein. Also the time treatment may be slightly increased when the cork pieces are of a size greater than given, say above about  $\frac{3}{4}$  inch. Thus, I have found it desirable in practicing the present invention to pretreat the cork by boiling the same in water for a period of about 10 to about 30 minutes to obtain a maximum absorption of moisture therein, this generally taking place in the first few minutes. By this pretreatment a maximum expansion of the cork pieces in a minimum time of treatment may be obtained and the extent of carbonization be, accordingly, reduced to a negligible amount, if any at all. I have also observed that in the preferred temperature range the volume change in the cork for all periods above about 40 seconds treatment is substantially negligible, and that the optimum expansion of the cork occurs in this period of treatment regardless of whether or not the cork has been pretreated as described or a cork material previously somewhat heat treated is employed. I would have it understood that while I prefer to initiate the present process with natural cork pieces, cork pieces which may have been somewhat expanded by other processes may be utilized and be given the benefits of the present process to the extent that their initial condition permits. In some cases with cork of this character it will be found desirable to reduce the total time of treatment to obtain the desired results. Moreover, it will be understood that the percentages of volume change given are based upon natural cork and that, accordingly, when a pre-expanded cork is subjected to the present

process it quite naturally may not have a total expansion within the optimum figures given.

It is sometimes found in the present process that small quantities of metal where a metallic bath is employed are mechanically carried out with the cork pieces even though such material does not adhere thereto. I have found that this metal may be easily separated from the cork when the expanded cork pieces are ground and screened for use and more readily by subjecting the ground cork to flotation in water in which case any metal immediately settles to the bottom where it may be removed. If the cork material is to be utilized in the manner described in my co-pending application aforesaid, in conjunction with an aqueous, fibrous suspension the ground, treated cork may be directly mixed therewith as the metal particles will settle to the bottom of the receptacle in which the cork and fiber are mixed and may readily be removed. Accordingly, the step of removing foreign metallic particles is an added feature of the present invention.

For a better understanding of the present invention the following examples are given which are not in any manner to be considered as limiting the present invention:

*Example No. 1*

A lead bath is fitted with a funnel dipping slightly beneath the surface of the lead; the end of the funnel is fitted through a delivery tube to a condenser. A small wire cage is made with handle attached which can be held beneath the surface of the lead by suitable supporting means, and under the funnel. The cage is partially filled with granulated natural cork preferably between  $\frac{1}{4}$  inch and  $\frac{1}{2}$  inch in size, allowing ample space in the cage for the material to expand without restriction. The cage containing the cork pieces is then held in the bath with the cork submerged for a period of about 40 seconds with the bath kept at a temperature of about 350° C. (662° F.). During this treatment volatile matter boils off through the lead and up through the funnel into the condenser where it is condensed and flows into a receiver. After 40 seconds the cage is removed from the lead and the treated cork pieces are taken from the cage. The operation is repeated until the desired quantity of treated cork is obtained. For the uses contemplated in my copending application aforesaid the treated cork pieces are then ground to a size preferably passing through a 12 mesh screen and in such condition the regranulated cork will have a density of about 2.15 pounds per cubic foot. The material is dark brown in color and while it grinds easily compared to natural cork, it is very springy and not at all brittle. About 17% of distillate is obtained based upon the weight of the natural cork and this is almost entirely aqueous with very little oil. The distillate is dark reddish brown, has a strong characteristic odor and acid reaction and becomes darker upon standing. While the lead of the bath does not adhere to the cork in the processing, small quantities may be carried out with the cork pieces mechanically. Such may be easily separated as described above by grinding and floating the cork in water. Any lead, of course, then immediately settles to the bottom of the water and is separated.

Where it is desired to obtain the treated cork product of the invention by a continuous procedure the raw material may instead of being placed in a wire cage be fed, as shown in the drawing, from a source of supply 10, to a feed

hopper 12, connected to a heating chamber 14, charged with molten lead to a level 16. The chamber 14, receives its heat from a furnace 18, situated below the bath and the chamber has a gas-tight cover or head 20, provided with an outlet 21, from which the volatiles of the cork material may be withdrawn and conveyed to a condenser, not shown, for further treatment to obtain the by-products thereof. Within the chamber is a conveying device consisting of a pair of sprockets 22, carried by suitable shafts supported on suitable trunnions and a chain or chains 24, operating immediately adjacent but not in the metallic bath. The chain carries a multiplicity of thin metallic L shaped plates 26, secured to the chain so that they project at right angles to the links thereof and dip into the metallic bath along the low run of the chain. The feed hopper is of a size capable of receiving a sufficient charge to last for a complete run and is provided with a gas-tight cover and port to prevent the escape of volatiles through this member. The low end of the hopper 12, has an opening 28, entering into the chamber 14, and through which the raw material drops upon the surface of the metallic bath and into operative contact with the plate members 26, of the continuous chain. In the drawing the sprockets are indicated to rotate in a counterclockwise direction so that the plates 26, act against the accumulated cork material on the surface of the bath and take a layer of such material along in passing down into the bath and through its length. Obviously, the side edges of the chain may be provided with suitable shields for preventing the escape of the cork pieces out the ends of the spaces formed between the plate members. It is preferred that the depth of the plates be such that only a single layer of cork particles be drawn by the plates below the surface of the bath.

At the opposite end of the chamber where the chain plates emerge from the bath a discharge port 30, is provided having its lower lip just above the level of the bath. The expanded cork granules as they emerge from the lead bath are pushed by the plates and directed through the discharge port 30, into a discharge hopper 32, where they are accumulated until a sufficient amount is collected for the next step. It will be understood, however, that the particles may be fed continuously to the next operating means if desired. Upon leaving the bath the cork pieces may take with them mechanically held particles of lead. In order to remove the lead the expanded cork pieces are now transferred, preferably by gravity, to a storage hopper 34, positioned above a conveyor 36 which carries the particles to a grinder 38, where the cork pieces are divided into the desired sizes and fed to a screen 40, which permits the desired sizes to pass therethrough and retains the oversize particles which are returned by the means 42, to the grinder for reprocessing. The particles passing through the screens are dropped into a separation tank 44 containing water and the lead particles having been loosened from the cork pieces in the grinding and screening process readily fall to the bottom of the tank where they may be recovered and returned to the bath, and the cork pieces float upon the surface of the liquid and are discharged through a port 46 by a paddle 48. The wet particles may be immediately transferred to a wet process tank for employment in making the products of my co-pending application aforesaid or the wetted particles may be dried and sent to storage. Ob-

viously the volatiles obtained in the processing may be collected and condensed for further treatment. It will be understood that the chain 24 may be driven through a variable speed drive so that its linear speed may be adjusted to give the cork pieces a predetermined period of submersion in the lead bath.

#### Example No. 2

In this example either apparatus and procedure as used in Example No. 1 may also be employed. The time of treatment of the cork pieces is, however, increased to three minutes and the metallic bath comprises a molten alloy consisting of 20% tin and 80% lead (melting point 572° F.). The temperature of the bath during the treatment is maintained at about 330° C. (626° F.). The expanded cork obtained in this case is not as springy as that in Example No. 1 and crushes more readily, but is not of a brittle nature. When ground to a size passing a 12 mesh screen the density is found to be 1.51 pounds per cubic foot. In this case about 40% distillate is obtained based upon the weight of the natural cork used. This distillate contains about 50% of aqueous material and the remainder is a waxy oily material which separates with difficulty. When treated with strong caustic, the oily material is dissolved and a yellowish brown wax is precipitated which can be separated. This waxy material decomposes when heated to its boiling point and from its general characteristics would seem to be related to the cork waxes, cerin and friedelin, more generally referred to as cork alcohols.

From the above examples it will be understood that various mediums may be employed for the cork treatment. Moreover, it will be understood that cork pieces, other than natural cork, for example, cork that has been partially expanded by other treatments, may be further processed in the described manner to obtain the additional benefits thereof of expansion and fungus growth resistance. It will be further seen that natural cork may be expanded by treatment in a metallic bath with the removal of up to 40% of volatile and decomposition volatile matter and with the production of a resilient, expanded, super lightweight product that is soft and rubbery, free from excess surface carbonization, non-brittle, and has a degree of springiness dependent upon the kind of treatment. It should be noted that the chemical action taking place in the cork during the process of the present invention is unique and differs from that taking place when using a retort described in my co-pending application aforesaid. In the latter procedure various aqueous and oil distillates are obtained as by-products but in the present process, while a similar aqueous distillate is obtained, it has only a slight amount of oil present and in addition a large amount of waxy material is collected. It is believed that this waxy material is more of a primary substance that may have direct uses as a waxy substance. The waxy material is relatively unstable and when subjected to distillation breaks down into the various oils obtained by the retort treatment of my prior application. It seems quite remarkable that this waxy substance will distill through the metallic bath without decomposition during the expansion treatment of the cork in view of its relative instability. Apparently the critical temperature range and the rapidity of expansion to which the cork is subjected necessitating only a short interval of treatment and the obviously rapid discharge of the volatiles re-

removed from the cork are responsible for the obtaining of the waxy substance which is apparently not otherwise obtained. While waxes have been extracted from cork by expensive solvent extraction, none has ever to my knowledge been obtained by heat treatment of cork. Accordingly, the processing for obtaining by-products such as the primary waxy substance constitutes a further and additional feature of the present invention.

From the foregoing description it will be seen that I have presented a new and novel process of expanding cork pieces, that I have produced a cork material of exceedingly low density and that may be non-brittle, soft, rubbery and springy; that I have discovered a procedure for producing cork distillates that eliminates steps heretofore found necessary in my prior procedures, and that I have discovered a process of obtaining cork pieces of exceptional low density that may or may not possess fungus growth inhibiting properties. The new process is simple, practical, readily controlled, and economical in its operation. It will be appreciated that various departures from the specifically disclosed procedure will occur to those skilled in the art without departure from the letter and spirit of the present invention. For example, the heat treatment may be carried out in several steps and the raw cork at the beginning of the process may not be a natural cork. Accordingly, it is desired that the present invention be construed to include all equivalents and as broadly as the following claims taken in conjunction with the prior art may follow. Whenever specific values are given for densities of the new cork product throughout the specification and in the claims, it is intended that these are densities of the cork when ground to a size passing a 12 mesh screen and retained on a 50 mesh screen. However, it is to be understood that fines of a size smaller than 50 and pieces greater than 12 are not outside the scope of the present invention, the figures given being intended solely as a guide for testing densities.

I claim:

1. The process of making low density cork pieces adapted for insulation and the like, comprising providing a multiplicity of cork pieces to be treated, submerging said cork pieces in and in direct contact with a liquid medium substantially non-absorbent and non-adherent with respect to cork, and having a temperature between 580° F. to 720° F. and maintaining said cork pieces in said liquid medium for a total period not exceeding about four minutes.

2. A process as in claim 1 wherein the temperature of the liquid medium is between about 620° F. to about 680° F.

3. A process as in claim 1 wherein the temperature of the liquid medium is between 620° F. to about 655° F.

4. A process as in claim 1 wherein the liquid medium is a molten metallic one.

5. The process of making low density cork pieces adapted for insulation and the like, comprising treating a multiplicity of cork pieces having a density not under about 5 pounds per cubic foot by submersion, in a condition in which the cork is free to expand without restriction, in and in direct contact with a molten lead bath having a temperature sufficiently high but not under 580° F. and not over 720° F. for a total period of time not exceeding about four minutes to obtain individual cork pieces having a density between about 1½ to 3 pounds per

cubic foot and substantially free from excessive surface carbonization and having a soft, resilient and rubbery character.

6. In the process of making low density regranulated cork adapted for insulation and the like, the steps comprising preparing cork pieces substantially under ¼ inch in size, submerging said pieces in and in direct contact with a molten metallic bath comprising lead having a temperature between about 620° F. to about 680° F., maintaining said pieces in the bath for a total period not exceeding about four minutes, whereby to effect a rapid expansion of said cork pieces with removal of volatiles including decomposition material, and grinding said cork pieces to a size passing through a number 12 mesh screen, said cork having a density between about 1½ to 3 pounds per cubic foot.

7. The process of making low density cork pieces adapted for insulation and the like, comprising submerging cork pieces substantially between ¼ to ½ inch in size, in a condition in which the cork is free to expand without restriction, in and in direct contact with a molten metallic bath having a temperature between about 620° F. to about 680° F. for a total period between about 40 seconds to about 3 minutes.

8. The process of making low density cork pieces adapted for insulation and the like, comprising submerging natural cork pieces in and in direct contact with a molten metallic bath having a temperature between about 620° F. to about 680° F. for a total period of time in the order of about 40 seconds to effect a rapid expansion of the cork pieces in amount exceeding about 200% by volume and loss of volatiles in amount not exceeding about 15% by weight of the natural cork.

9. The process of making low density cork pieces adapted for insulation and the like, comprising submerging natural cork pieces in and in direct contact with a molten metallic bath having a temperature between about 620° F. to about 680° F. for a total period of time not exceeding about 4 minutes, whereby to effect a rapid expansion of the cork pieces in an amount at least between 200 to 375% by volume and a removal of volatiles and decomposition material in amount exceeding 15% but substantially no greater than 40% by weight of the natural cork.

10. The process of making low density regranulated cork comprising preparing natural cork granules between about ¼ inch to about ½ inch in size, submerging said cork granules in and in direct contact with a liquid metallic bath comprising lead maintained at a temperature between about 620° F. to about 680° F., treating said cork granules for a total period of submergence between about 40 seconds to about 4 minutes to effect a rapid expansion of the cork granules together with removal of volatiles and decomposition material, whereby to obtain individual cork granules having a volume increase between about 200 to 375% and a loss of volatiles and decomposition material between about 15% to about 40% by weight of the natural cork, and comminuting said cork granules to a size passing a 12 mesh screen to produce regranulated cork having a density between about 1½ to about 2½ pounds per cubic foot.

11. The process of making low density cork pieces adapted for insulation and the like, comprising treating cork pieces in boiling water to effect a partial absorption of moisture therefrom,

submerging said water treated cork pieces containing said absorbed water in and in direct contact with a molten metallic bath maintained at a temperature between about 620° F. to about 680° F., and treating said cork pieces in said bath for a total period between about 20 seconds to about 3 minutes.

12. The process of making low density cork pieces adapted for insulation and the like, comprising heat treating natural cork pieces having a density between 6 to 8 pounds per cubic foot to obtain cork pieces of a density between 5 to 6 pounds per cubic foot, and submerging said pretreated cork pieces in and in direct contact with a molten metallic bath maintained at a temperature between 580° F. to 720° F. for a total period not exceeding about 4 minutes to obtain individual cork pieces having a density between about 1½ to 2½ pounds per cubic foot.

13. The process of obtaining cork waxed comprising treating comminuted cork in and in direct contact with a molten metallic bath main-

tained at a temperature between about 580° F. to 720° F., collecting the volatiles and decomposition matter given off from said cork and condensing and separating the waxy material from said condensate.

14. The process of making low density cork pieces adapted for insulation and the like, comprising providing a multiplicity of cork pieces to be treated, submerging said cork pieces in and in direct contact with a molten metallic medium substantially non-absorbent and non-adherent with respect to cork and having a temperature between 580° F. to 720° F., maintaining said cork pieces in said medium for a total period not exceeding about 4 minutes to obtain a rapid expansion of said cork pieces together with a loss of volatile and decomposition matter, agitating said cork pieces to loosen any mechanically held metal, and depositing said cork pieces in water to effect separation of said cork pieces and metal.

CHARLES H. SCHUH.